# EUROPEAN PATENT SPECIFICATION

(11) **EP 0 819 788 B1**
(45) Date of publication and mention of the grant of the patent: **07.05.2003**
(21) Application number: 97111983.9
(22) Date of filing: 14.07.1997
(51) Int. Cl.: D04H 1/46, D06M 15/53, D06M 15/507, C03C 25/00

(54) **Needling aid for producing needle felts, a needle felt produced by using it, and a method for production thereof**
Verfahrenshilfsmittel für ein Nadelfilz, ein unter Anwendung dieses Verfahrenshilfsmittels hergestelltes Nadelfilz und Verfahren zu dessen Herstellung
Aide d'aiguilletage pour le production de feutres aiguilletés, feutre aiguillete fabrique utilisant cette aide et procédéde production

(30) Priority: 15.07.1996 DE 19628477
(43) Date of publication of application: 21.01.1998
(73) Proprietor: SAINT-GOBAIN ISOVER, 92400 Courbevoie (FR)
(72) Inventor: Amannt, Gerald, 69259 Wilhelmsfeld (DE); Holstein, Wolfang, Dr., 35315 Homburg (DE)
(74) Representative: Kuhnen & Wacker

(56) References cited:
- EP-A- 0 363 707
- EP-A- 0 638 629
- US-A- 3 913 191
- US-A- 4 654 235

## Description

The present invention concerns a needling aid for producing needle felts of mineral wool in accordance with claim 1, and its use for producing a needle felt in accordance with claim 10.

Needle felts are particularly suited for thermal insulation in household appliances, for instance in ovens and cookers as well as in industrial muffle-type furnaces.

For needle-punching mineral wool felts, a needling aid, or finishing agent, must be applied onto the fibers as an additive. Such finishing agents are variously produced on the basis of mineral oils, natural oils or fatty acid derivatives. The finishing agent is required for making the fibers smooth and reducing their mutual friction during the needle-punching process to prevent breakage or rupturing of the fibers during needle-punching as far as possible. The finishing agent must furthermore be capable of binding dusts released during the production process, to thereby permit processing and utilisation of the needle felt in the absence of any additional dust protection measures.

Typically such finishing agents are sprayed onto the fibers in the chute of a fiberising machine for the molten glass material, or directly onto the felt mat. This implies a tradeoff with respect to viscosity inasmuch as sufficient spraying must be ensured on the one hand, whereas a material having a sufficiently high viscosity must be retained following evaporation of the carrier material in order to guarantee the above mentioned advantages for the needle-punching process.

Formerly, particularly suited finishing agents were therefore lubricating oils and lubricants on mineral oil basis. A drawback of utilising such substances as a needling aid did, however, reside in the fact that considerable amounts of one or several emulsifiers had to be added for producing an aqueous dispersion or emulsion to thereby prevent phase separation into mineral oil phase and aqueous phase from occurring even as early as in the storage container of the finishing agent dispenser. To this end, particularly alcohol, alkoxylates and/or nonylphenol were used as emulsifiers in the past, however these had the facultative disadvantage of decomposing and thereby releasing formaldehyde upon being heated in needle felts which are utilised for thermal insulation of household appliances, e.g. ovens and cookers, and industrial muffle-type furnaces.

It has, however, also been found in the past that even if needle felts were subjected to thermal after-treatment following needle-punching in order to remove the needling aid - not to mention the increased expense in terms of energy and costs - residual finishing agent and in particular residues of the emulsifiers contained in it may still cause malodors or even the release of formaldehyde at the location of the final user. This is particularly true for the first few weeks of operation of ovens and cookers.

In order to avoid these difficulties, various approaches were tried in the prior art. Thus it was attempted e.g. to disperse mineral oil products in water via a high-pressure dispersion mixing device in such a way as to do away with the addition of emulsifier. This did, however, amount to a major technical effort on the one hand and did not provide the desired results on the other hand.

Another approach to avoid this problem was based on the fact that, in accordance with DE-PS-42 01 868, a thixotropising additive is used with a standard finishing agent on a fatty acid polyglycolester basis. Such a thixotropising additive has the advantage of having a high viscosity at rest and thus holding the fiber loops in their anchoring positions achieved by the needle-punching process, whereas the presence of a low dynamic viscosity results in good needle-punching properties and a good lubricating effect. Owing to a high degree of fluidity while the needles are acting on the felt to be needle-punched, it is possible to have to add only small quantities of needling aid, whereby malodors under the effect of heat are correspondingly diminished.

It is, however, a drawback of this finishing agent, or of these needle felts of the prior art, that malodors and thermal decomposition products, which are particularly undesirable in the field of household appliances, continue to occur.

Starting out from this prior art, it is therefore an object of the present invention to furnish a needling aid for producing a needle felt, which practically does not release any toxic decomposition products, in particular any formaldehyde, at temperatures occurring in the heat insulation particularly of ovens and cookers.

With respect to a needling aid, this object is achieved through the characterising features of claim 1. With respect to a needle felt, the above object is achieved by the features of claim 10.

Since the needling aid of the invention contains an aqueous dispersion of at least one at least partly halogenated polymer and an alcohol, on the one hand there result excellent oil-like finishing agent properties owing to the molecular conditions, and on the other hand those are chemically inert, halogenated polymers which, as a rule, resist thermal decomposition or are otherwise decomposed into nontoxic products. Such partly halogenated polymers are selected from the group consisting of:
halogenated polyethers, fluorated polyethers, in particular perfluorated polyethers, chlorated polyethers, in particular perchlorated polyethers, brominated polyethers, in particular perbrominated polyethers;
halogenated polyesters, fluorated polyesters, in particular perfluorated polyesters, chlorated polyesters, in particular perchlorated polyesters, brominated polyesters, in particular perbrominated polyesters; and
halogenated polyols, fluorated polyols, in particular perfluorated polyols, chlorated polyols, in particular perchlorated polyols, brominated polyols, in particular perbrominated polyols;
as well as mixtures thereof.

The terms "perfluorated", "perchlorated" and "perbrominated" are meant to indicate that practically each hydrogen atom within the polymer is replaced by a corresponding halogen atom, wherein one or both terminal groups can be not halogenated or partly halogenated.

Formaldehyde could be detected neither in the chute nor in the final needle felt which was exposed to a temperature of up to 500°C for approx. 1 hour.

Under practical conditions, the perfluorated polyethers in accordance with claim 4 have hitherto turned out to be particularly suitable needling aids as they bring about extremely favorable sliding properties between the fiber loops during needle-punching on the one hand, and as practially all hydrogen atoms within the polyether system are replaced by fluorine atoms on the other hand, such perfluorated polyethers are chemically inert and also thermally resistant.

The perfluorated polyether in accordance with claim 5 has been found to be a particularly preferred embodiment of a needling aid, which is commercially available e.g. under the designation Fomblin FE 20C.

Adding a sterically inhibited alcohol, preferably t-butanol, to the needling aid in addition to the halogenated polymer in accordance with claims 6 and 7 has the advantage that the dispersion is stabilised by it, with the t-butanol, having a boiling point of approx. 80°C, instantaneously evaporating in the chute without furthermore leaving behind any decomposition products. Addition of such an alcohol stabilises the dispersion or emulsion in water of the polymer used.

A particularly preferred needling aid is one in accordance with claim 8, wherein the dispersion is present as an aqueous micro-emulsion. Such micro-emulsion has the advantage that it presents homogeneous distribution of the utilised halogenated polymer in water even without any costly mixing processes, such that the obtained good results are also reproduceable in subsequent lots.

Upon application onto the fibers of the mineral wool, in particular glass wool, the aqueous emulsion preferably has a concentration of approx. 0.1 to 0.5% (wt.) of halogenated polymer and approx. 0.05 to 0.45% (wt.) of t-butanol. At these final concentrations during application onto the mineral wool, only small quantities of needling aid are required to obtain the properties desired for needle-punching.

Owing to the small amounts of needling aid according to the invention, the incurred costs are reasonable compared with those of conventional finishing agents.

In claim 10 the use of a needling aid according to any one of claims 1 to 9 is claimed to produce a needle felt of mineral wool. An important advantage of the needle felt according to the invention resides in the fact that for the first time a formaldehyde-free needle felt is available which will not release formaldehyde even under a high thermal load of up to approx. 500°C in accordance with claim 11.

The needle felts according to the invention are therefore well suited for thermal insulation in household appliances, in particular ovens and cookers, inasmuch as they produce neither unpleasant smells nor toxic decomposition products upon initial operation at the location of the end user.

It should be noted in the framework of the present invention that the needling aid according to the invention is suited for needle-punching mineral wool, particularly, however, having the form of glass wool.

Further advantages and features of the present invention result from the description of an embodiment.

### Example

For producing a needling aid composition according to the invention, an aqueous micro-emulsion of a perfluoropolyether commercially available under the designation "Fomblin FE 20C" was used. This emulsion has a polymer content of approx. 20% (wt.) and is stabilised with approx. 18% (wt.) of t-butanol.

The perfluorated polyether used in the example had the following general formula:

CF₃-(O-CF(CF₃)-CF₂)ₙ-(O-CF₂)ₘ-O-CF₂-R,

with R = -COO⁻ NH₄⁺ or -C(OH)₂-CF₃, and n and m being integers with n/m approx. 20 to 40.

For producing a practically applicable solution or dispersion, the commercially available solution is diluted with water to a polymer content of approx. 12% (wt.). In the preparing vessel of the needle felt line, 3 kg of the 12% emulsion are then added into 250 kg of water and mixed by means of a propeller agitator.

This solution containing a final concentration of approx. 0.15% (wt.) polymer, e.g. perfluoropolyether, was then sprayed onto e.g. a glass wool felt, and the latter conveyed under a needle bench and subjected to a needle-punching process. As an alternative, the needling aid of thet above example is sprayed directly onto the fibers in the chute.

A needle felt produced from glass wool in this manner has a bulk density of approx. 50 kg/m³ and a thickness of approx. 17 mm.

The needle felts thus produced were subjected to thermal load at approx. 250°C in a standard kitchen in accordance with DIN 44971 in previously annealed cookers, and possibly produced decomposition products were analysed.

Here it was found that on the one hand no toxic products were produced at all, in particular neither formaldehyde nor hydrogen fluoride could be detected in the oven exhaust air.

Thus annealing of the needling aid subsequent to the needle-punching process, as it is frequently required with conventional finishing agents, is not necessary. The needle felts of the present invention therefore have excellent suitability for use in household appliances such as ovens or cookers as a heat insulation material, as it was also found in tests with such apparatus that malodors occurred neither upon initial use nor upon use over a period of several weeks, and that toxic products are not released into the surrounding atmosphere.

## Claims

1. Needling aid for producing needle felts of mineral wool,
**characterised in that**
it contains an aqueous dispersion of at least one at least partly halogenated polymer which is selected from the group consisting of:
halogenated polyethers, halogenated polyesters, halogenated polyols, as well as mixtures thereof, and an alcohol.

2. Needling aid according to claim 1,
**characterised in that** the polyethers, polyesters and/or polyols are fluorinated, chlorinated and/or brominated.

3. Needling aid according to claim 2,
**characterised in that** the polyethers, polyesters and/or polyols are perfluorinated, perchlorinated and/or perbrominated.

4. Needling aid according to claim 3, **characterised in that** it contains a perfluorinated polyether.

5. Needling aid according to claim 4, **characterised in that** the perfluorinated polyether has the following general formula:
CF₃-(O-CF(CF₃)-CF₂)ₙ-(O-CF₂)ₘ-O-CF₂-R
with R = -COO⁻NH₄⁺ or -C(OH)₂-CF₃, and n and m being integers with n/m approx. 20 to 40.

6. Needling aid according to any one of claims 1 to 5, **characterised in that** the alcohol is a sterically inhibited alcohol.

7. Needling aid according to claim 6, **characterised in that** the alcohol is t-butanol.

8. Needling aid according to any one of claims 1 to 7, **characterised in that** the dispersion is present in the form of an aqueous micro-emulsion.

9. Needling aid according to any one of claims 1 to 8, **characterised in that** the aqueous emulsion has the following concentrations upon application onto the fibers of the mineral wool:
approx. 0,1 to 0,5 % (wt.) of polymer
approx. 0,05 to 0,45 % (wt.) of t-butanol.

10. Use of a needling aid according to any one of claims 1 to 9 for producing a needle felt of mineral wool.

11. Use according to claim 10, **characterised in that** the needle felt produced does not liberate any formaldehyde upon being heated to approx. 500 °C.

12. Use according to claim 10 or 11, **characterised in that** a needling aid according to any one of claims 1 to 9 is added to a felt mat, and the latter is then needle punched.

## Patentansprüche

1. Nadelhilfsmittel zur Herstellung von Nadelfilzen aus Mineralwolle, **dadurch gekennzeichnet, daß** es eine wäßrige Dispersion aus mindestens einem zumindest teilweise halogenierten Polymer umfaßt, das ausgewählt ist aus der Gruppe bestehend aus: halogenierten Polyethern, halogenierten Polgestern, halogenierten Polyolen ebenso wie deren Mischungen, und einem Alkohol.

2. Nadelhilfsmittel nach Anspruch 1, **dadurch gekennzeichnet, daß** die Polyether, Polyester und/oder Polyole fluoriert, chloriert und/oder bromiert sind.

3. Nadelhilfsmittel nach Anspruch 2, **dadurch gekennzeichnet, daß** die Polyether, Polyester und/oder Polyole perfluoriert, perchloriert und/oder perbromiert sind.

4. Nadelhilfsmittel nach Anspruch 3, **dadurch gekennzeichnet, daß** es einen perfluorierten Polyether enthält.

5. Nadelhilfsmittel nach Anspruch 4, **dadurch gekennzeichnet, daß** der perfluorierte Polyether die folgende allgemeine Formel aufweist:
CF₃-(O-CF(CF₃)-CF₂)ₙ-(O-CF₂)ₘ-O-CF₂-R
wobei R = -COO⁻NO₄⁺ oder -C(OH)₂-CF₃, und n und m ganze Zahlen sind, wobei n/m ungefähr 20 bis 40 ist.

6. Nadelhilfsmittel nach einem der Ansprüche 1 bis 5, **dadurch gekennzeichnet, daß** der Alkohol ein sterisch gehinderter Alkohol ist.

7. Nadelhilfsmittel nach Anspruch 6, **dadurch gekennzeichnet, daß** der Alkohol t-Butanol ist.

8. Nadelhilfsmittel nach einem der Ansprüche 1 bis 7, **dadurch gekennzeichnet, daß** die Dispersion in Form einer wäßrigen Mikroemulsion vorliegt.

9. Nadelhilfsmittel nach einem der Ansprüche 1 bis 8, **dadurch gekennzeichnet, daß** die wäßrige Emulsion die folgenden Konzentrationen aufweist, nachdem sie auf die Mineralwollfasern aufgebracht wurde:
ungefähr 0,1 bis 0,5 % (Gew.) Polymer
ungefähr 0,05 bis 0,45 % (Gew.) t-Butanol

10. Verwendung eines Nadelhilfsmittels nach einem der Ansprüche 1 bis 9 zur Herstellung eines Nadelfilzes aus Mineralwolle.

11. Verwendung nach Anspruch 10, **dadurch gekennzeichnet, daß** der erzeugte Nadelfilz kein Formaldehyd abgibt, nachdem er auf ungefähr 500 °C erwärmt wurde.

12. Verwendung nach einem der Ansprüche 10 oder 11, **dadurch gekennzeichnet, daß** das Nadelhilfsmittel nach einem der Ansprüche 1 bis 9 der Filzmatte zugegeben wird und letztere dann genadelt wird.

## Revendications

1. Aide d'aiguilletage pour la production de feutres aiguillés en laine minérale, **caractérisée en ce qu'**elle contient une dispersion aqueuse d'au moins un polymère au moins partiellement halogéné qui est choisi dans le groupe composé de :
polyéthers halogénés, polyesters halogénés, polyols halogénés, ainsi que des mélanges de ceux-ci, et un alcool.

2. Aide d'aiguilletage selon la revendication 1, **caractérisée en ce que** les polyéthers, polyesters et/ou polyols sont fluorés, chlorés et/ou bromés.

3. Aide d'aiguilletage selon la revendication 2, **caractérisée en ce que** les polyéthers, les polyesters et/ou les polyols sont perfluorés, perchlorés et/ou perbromés.

4. Aide d'aiguilletage selon la revendication 3, **caractérisée en ce qu'**elle contient un polyéther perfluoré.

5. Aide d'aiguilletage selon la revendication 4, **caractérisée en ce que** le polyéther perfluoré a la formule générale suivante :
CF₃- (O-CF(CF₃)-CF₂)ₙ-(O-CF₂)ₘ-O-CF₂-R
Dans laquelle R = -COO-NH₄⁺ ou -C(OH)₂-CF₃, et n et m étant des nombres entiers avec n/m étant approximativement égal à 20 à 40.

6. Aide d'aiguilletage selon l'une quelconque des revendications 1 à 5, **caractérisée en ce que** l'alcool est un alcool stériquement inhibé.

7. Aide d'aiguilletage selon la revendication 6, **caractérisée en ce que** l'alcool est du t-butanol.

8. Aide d'aiguilletage selon l'une quelconque des revendications 1 à 7, **caractérisée en ce que** la dispersion est présente sous la forme d'une micro-émulsion aqueuse.

9. Aide d'aiguilletage selon l'une quelconque des revendications 1 à 8, **caractérisée en ce que** l'émulsion aqueuse a les concentrations suivantes lors de l'application sur les fibres de la laine minérale :
environ 0,1 à 0,5% en poids de polymère
environ 0,05 à 0,45% en poids de t-butanol

10. Utilisation d'une aide d'aiguilletage selon l'une quelconque des revendications 1 à 9 pour produire un feutre aiguilleté de laine minérale.

11. Utilisation selon la revendication 10, **caractérisée en ce que** le feutre d'aiguilletage produit ne libère aucun formaldéhyde lors d'un réchauffement à environ 500°C

12. Utilisation selon les revendications 10 ou 11, **caractérisée en ce qu'**une aide d'aiguilletage selon l'une quelconque des revendications 1 à 9 est ajoutée à un tapis de feutre, et celui-ci est ensuite aiguilleté.
